

## UNITED STATES PATENT OFFICE

MAURICE H. ARVESON, OF HAMMOND, INDIANA, ASSIGNOR TO STANDARD OIL COMPANY (INDIANA), OF CHICAGO, ILLINOIS, A CORPORATION OF INDIANA

LEAD MAHOGANY SOAP LUBRICANT AND METHOD OF PREPARING SAME

No Drawing.

Application filed May 12, 1930. Serial No. 451,884.

This invention relates to an improved method and lubricant for the commercial preparation of lead mahogany soap in a form suitable for use as a lubricant.

6 The expression "mahogany" has the same significance in this specification as it does in the petroleum industry. It is a generic name for the preferentially oil soluble radicals formed by the treatment of hydrocarbon oil with strong sulfuric acid in the preparation 10 of "white oils".

The object of my invention is to provide an improved process for preparing lead mahogany soaps on a commercial scale, using 15 petroleum hydrocarbon solvents. A further object is to provide an improved lubricant, combining the desirable qualities of lead mahogany soap and oil in a new combination of these substances. A further object is to 20 provide a process for removing salts and other impurities from lead mahogany soap and for making a soap which is stable and from which there will be no separation of lead oxide or other salts. A further object is to 25 provide an improved sequence of steps and regulation of proportions whereby clean separation of lead mahogany soap from salts and other impurities can be effected without a loss of yield and without the formation of 30 objectionable emulsions. Other objects will be apparent as the detailed description of my invention proceeds.

When oils, which have been treated with strong sulfuric acid, are neutralized with sodium hydroxide, oil soluble sodium mahogany soaps are formed, which may be extracted with naphtha. My invention contemplates the conversion of this sodium soap into a lead soap and the separation of lead mahogany 40 soap from its reaction products. The features of this process are:

1. The use of oil as a diluent for reaction products prior to the naphtha extraction of the lead soap.
2. The reduction of the water content prior

to the addition of said naphtha, for preventing emulsification.

3. The use of naphtha as a diluent without throwing the lead mahogany soap into the water layer.

4. The subsequent addition of water for removing impurities.

5. The final removal of solid and aqueous impurities by the addition of naphtha.

On a commercial scale it is extremely difficult to separate reaction products from lead mahogany soap, but I have discovered that by carefully regulating volumetric proportions in a definite sequence of steps I can prepare a lead mahogany soap which is free from deleterious impurities and which is combined with oil in a unique manner to form excellent lubricant for gears or for general use where high rubbing pressures are applied to relatively small surfaces. The invention will be more clearly understood from the detailed description of a preferred embodiment.

The treatment of petroleum oils with concentrated sulfuric acid to produce "white oils" is well known. It forms no object of the present invention and it therefore will not be described in detail. When the acid treated oil has been neutralized with sodium hydroxide, a sodium mahogany soap is formed which may be extracted with alcohol and purified. In my process I may start with what is technically known as Grade A sodium mahogany soap which consists of 70% soap, 20% oil, 3 to 5% water, and 5 to 8% occluded salts.

A solution of lead acetate is prepared, the amount being calculated to give an excess of about 40 to 50% (calculated from the sodium content of the soap.) The lead acetate solution, which is dissolved in a volume of water slightly less than the volume of sodium content of the soap). The lead acetate soap in a heated vessel by stirring. The temperature is maintained slightly above the boiling point of water, since the object of this step is to remove a large amount of water

from the mixture. If water is not removed at this point, the lead mahogany soap will form an emulsion therein when naphtha is added, and a separation of the desired end products will be impossible. If too much water is evaporated at this point, the mixture will become resinous and insoluble in oil, water or naphtha. It is essential, therefore, that the final water content at this time should be between 15 and 35%.

When the reaction products have been treated and agitated until its water content is only from 15 to 35%, I add, with continued stirring, two volumes of oil to the mixture (the original volume of sodium mahogany soap being taken as a unit volume.) The properties of the oil have a marked influence on the remaining steps of the process and on the quality of the finished product. I prefer to use a heavy over-head lubricating oil, having a viscosity of 105 to 115 Saybolt at 210° F. (this oil being commercially known as #60 Polarine). I have discovered that the addition of oil is essential to effect a satisfactory separation and I prefer to use two volumes of oil because this quantity gives most satisfactory results and at the same time makes it possible to obtain a high lead content in the finished product.

After oil has been added to the mixture, it is again heated and agitated until the water content is reduced to from 1 to 20%, preferably from 2 to 8%. The mixture is then allowed to cool and about 10 to 15% of naphtha is mixed with it. If the water content is too high when the naphtha is added, a difficult emulsion is formed and subsequent separation is practically impossible. I have found that about 11% of naphtha gives excellent results under the circumstances herein set forth.

After the naphtha has been added, the mixture is diluted with an amount of water equal to the combined volume of soap, oil and naphtha. When the water is added at this stage no serious emulsion is formed and substantially all water soluble salts and impurities, such as lead acetate, lead sulfate, sodium acetate, sodium sulfate, etc. are removed from the oil, soap and naphtha mixture. After a thorough agitation, this mixture is allowed to settle, and when a clear line of demarcation appears between the oily and aqueous layers, the upper layer of oil, soap and naphtha diluent is decanted or siphoned from the aqueous layer.

The oil, soap and naphtha mixture is further diluted with naphtha so that the total naphtha content is about 33% of the mixture. This last step removes the occluded salts and water remaining in the oil layer, and renders the solution bright in color. It is extremely important that all salts and impurities be removed from the soap and the last steps of this process should be repeated.

if the mixture is cloudy at this point. When the upper layer is bright, it is removed and concentrated preferably by steam distillation. If the last naphtha layer is not bright, the heated soap mixture will form a stiff, 70 tough, apparently irreversible-jell.

When naphtha is removed from the finished product there remains a composition comprised of lead mahogany soap and lubricating oil. This mixture is of light red color 75 and may be almost transparent. Its viscosity is from about 200 to 500 Saybolt at 210° F. and it has a lead content of from 3½ to 5%.

This composition is an exceptional effective lubricant for rear axles of automobiles 80 and for other uses where any rubbing friction at extremely high pressure is encountered.

While I have described my invention in detail, it is understood that I do not limit 85 myself to the specific oils or to temperatures, proportions, etc. except as defined by the appended claims; the viscosity of the finished product may be varied by the use of different diluent oils, and the consistency of the soap 90 may be varied by use of sodium mahogany soaps from different sources. A special feature of my invention is the fact that my finished lead soap is free from solid impurities 95 or from potential impurities. (Unstable substances which may later break down to give solid impurities.) This is particularly important in the lubrication of bearings where solids separating from a lubricant might cause corrosion, and jamming in delicate 100 mechanism.

I claim:

1. A lubricant comprising lead mahogany soap substantially free from salts and impurities and a lubricating oil substantially free 105 from salts and impurities.

2. A lubricant comprising a lubricating oil and a lead mahogany soap substantially free from salts and impurities, the lead content 110 of said lubricant being about 3½%.

3. The method of preparing a lubricant comprising lead mahogany soap and oil substantially free from salts and impurities which comprises adding lubricating oil to a mixture of lead mahogany soap, water and impurities, reducing the water in said mixture to an amount below 20%, diluting the mixture with naphtha, and mixing water with the diluted mixture for separating the salts and impurities. 115

4. The method of making lead mahogany soap which comprises mixing sodium mahogany soap with lead acetate and water, reducing the water content to 15 to 35%, adding lubricating oil to said mixture, further reducing the water content to about 5%, adding about 10 to 15% naphtha, adding an amount of water equal in volume to the volume of the mixture, separating the oily layer from the aqueous layer, removing the oc- 120 125 130

cluded impurities from the oily layer, and distilling the naphtha therefrom.

5. The method of removing impurities from a mixture of said impurities with lead 6 mahogany soap and oil which comprises reducing the percentage of water to an amount of from 1% to 20% prior to the addition of diluent naphtha, diluting the mixture with naphtha, adding water to the diluted 10 mixture, and mechanically separating the resulting aqueous phase from the oil phase.

Signed this 29th day of April, 1930, at Whiting, in the county of Lake, State of Indiana.

15 MAURICE H. ARVESON.

#### CERTIFICATE OF CORRECTION.

Patent No. 1,871,942.

August 16, 1932.

MAURICE H. ARVESON.

It is hereby certified that error appears in the printed specification of the above numbered patent requiring correction as follows: Page 1, line 86, strike out the syllable and words "dium content of the soap). The lead ace." and insert instead sodium mahogany soap, is mixed with said; and that the said Letters Patent should be read with this correction therein that the same may conform to the record of the case in the Patent Office.

Signed and sealed this 22nd day of November, A. D. 1932.

(Seal)

M. J. Moore,  
Acting Commissioner of Patents.

cluded impurities from the oily layer, and distilling the naphtha therefrom.

5. The method of removing impurities from a mixture of said impurities with lead 6 mahogany soap and oil which comprises reducing the percentage of water to an amount of from 1% to 20% prior to the addition of diluent naphtha, diluting the mixture with naphtha, adding water to the diluted 10 mixture, and mechanically separating the resulting aqueous phase from the oil phase.

Signed this 29th day of April, 1930, at Whiting, in the county of Lake, State of Indiana.

15 MAURICE H. ARVESON.

#### CERTIFICATE OF CORRECTION.

Patent No. 1,871,942.

August 16, 1932.

MAURICE H. ARVESON.

It is hereby certified that error appears in the printed specification of the above numbered patent requiring correction as follows: Page 1, line 86, strike out the syllable and words "dium content of the soap). The lead ace." and insert instead sodium mahogany soap, is mixed with said; and that the said Letters Patent should be read with this correction therein that the same may conform to the record of the case in the Patent Office.

Signed and sealed this 22nd day of November, A. D. 1932.

(Seal)

M. J. Moore,  
Acting Commissioner of Patents.

45

50

55

60

65

**CERTIFICATE OF CORRECTION.**

**Patent No. 1,871,942.**

**August 16, 1932.**

**MAURICE H. ARVESON.**

It is hereby certified that error appears in the printed specification of the above numbered patent requiring correction as follows: Page 1, line 86, strike out the syllable and words "dium content of the soap). The lead ace." and insert instead sodium mahogany soap, is mixed with said; and that the said Letters Patent should be read with this correction therein that the same may conform to the record of the case in the Patent Office.

Signed and sealed this 22nd day of November, A. D. 1932.

**(Seal)**

**M. J. Moore,  
Acting Commissioner of Patents.**